

## UNITED STATES PATENT OFFICE

ALBERT C. FISCHER, OF CHICAGO, ILLINOIS, ASSIGNOR TO THE PHILIP CAREY MANUFACTURING COMPANY, A CORPORATION OF OHIO

## CONSTRUCTIONAL MATERIAL

No Drawing. Application filed August 15, 1927, Serial No. 213,184. Renewed July 14, 1930.

This invention relates to constructional material, such as, roofing material; insulating material, tapes, shingles, packing and the like.

5 The object of my present invention is to provide such constructional materials with an adhesive coating which is normally sticky or tacky to the touch and which lastingly maintains this mastic condition whereby the 10 material may be packed and stored for long periods of time without losing its tackiness and may be transported to its place of installation and used in such tacky condition without further treatment.

15 A further object of my invention resides in the application of this normally lastingly adhesive, sticky to the touch, to sheets or strips of carrier material, hereinafter called vehicles, so that when rolled into package 20 form or placed face to face in contact with a similar sheet for packing and storing and transportation, they may be unrolled or pulled apart readily without tearing or damaging, and can be installed in tacky condition. 25 In this instance the tacky coating permits the facile separation of the contacting vehicle surfaces, the line of cleavage passing through the mastic itself. The vehicle thus provided with a lasting adhesive, mastic coating is particularly adapted to act as a packing for various types of installation, not only because of the waterproofing quality of the mastic but also because of its pronounced and 30 lasting quality of adhesiveness and further because of its plasticity.

35 A further object of my invention resides in saturating a vehicle with a slow-drying, viscous adhesive, such for example as a bituminous substance, preferably a high melting point bituminous substance, combined with an oil or combination of oils.

40 In the present invention the vehicle may consist of sheets, strips, or slabs of tar paper, felt, fabric, fibers or other preferred material.

45 If preferred, the saturant of the vehicle

may be a slow-drying adhesive. Gilsonite or other more bituminous substances may be used in varying proportions (for example, from 10 to 20 per cent) with a non-drying oil such as castor oil (90 to 80 per cent). If a 50 blown castor oil is used, the proportion may range as high as 95 per cent of blown castor oil with 5 per cent of bitumen, gilsonite, Texas, or Trinidad. It may be necessary in 55 some cases to heat under pressure in order to secure union. It will be understood, of course, that the percentages referred to are merely illustrative and will vary under varying 60 conditions. Other oils and other bituminous substances may be used, in which cases the proportions will be subject to considerable variation. For instance, 15 per cent of bitumen, 75 per cent of castor oil and 10 per cent of rape-seed oil may be united by gradual 65 heating. The saturant may also be a combination of two or more of the following substances: cotton-seed oil, cotton-seed oil foot's, or pitch, and semi-liquid bituminous 70 substances of various consistencies.

75 The saturant may be the combination of a bituminous substance and a vegetable oil heated and combined at high temperature producing a viscous saturant. Gilsonite, Texas or other high melting bituminous substances may be used in varying proportions from 10 to 20 per cent, and a viscous oil, such as castor, where union with other oils is not desirable 80 to 90 per cent. If a blown castor oil is used the proportions may be as high as 80 5 per cent bitumen, gilsonite, Texas or Trinidad and 95 per cent blown castor oil. It may be necessary in some cases to heat under pressure in order to secure union.

85 The coating with which the vehicle is thus saturated on either one or both sides preferably comprises a slow-drying, tacky bituminous substance or combination of two or more, which approximates the following 90 specifications, or may be more or less fluid.

1. The consistency at 77 degrees F. should be below 7.0.
  2. The susceptibility factor should be as low as possible, preferably under 25.
  3. The ductility at 77 degrees F. should be as high as possible and preferably over 25 centimeters.
  4. Fusing point by K & S method should be between 80 degrees and 100 degrees F.
  5. It should appear tacky and adhesive at normal temperature and retain this property as long as possible on exposure to air.
- This formula is merely a standard and other formulas more or less fluid may be used with or without a suitable filler as a flow retarder, or the flow tendency may be stopped by using a non-flowing gummy substance in combination.
- It will be understood that my invention contemplates constructional material, the adhesiveness of which serves to hold said material in place in distinction to other materials which involve the use of pitch, or other material, mopped on at the time of assembling the material. This is especially true in the application of the invention to roofing sheets, for the purpose of holding the sheets of roofing material in place. It will be understood that after two sheets of building material according to the present invention have been separated, the adhesive surface of one sheet will be placed in contact with the non-adhesive surface of another sheet. The adhesive or mastic will cause a union with non-adhesive surfaces to which it is applied, which union may be made very excellent by means of rolling and which will improve in the course of time.
- It will also be understood that if it should be found that the adhesive surface of a sheet should become dried out, a solvent such as toluol, benzol, kerosene, or cotton oil, may be used to bring the sheet back into adhesive state.
- The subject matter of this application has been withdrawn from my prior patent, No. 1,550,310, issued August 18, 1925.
- I claim:
1. Constructional material comprising a vehicle saturated with a slow-drying adhesive composed of a bituminous substance and a non-drying oil, said saturated vehicle being coated with a waterproofing, mastic substance, normally sticky to the touch and lastingly adhesive.
  2. Constructional material comprising a vehicle saturated with high melting point bituminous material and a viscous oil, said saturated vehicle being coated with a waterproofing, mastic substance, normally sticky to the touch and lastingly adhesive.
  3. Constructional material comprising a vehicle saturated with a composition of bituminous material and a non-drying oil, and coated with a waterproofing, mastic, normally sticky to the touch and lastingly adhesive.
4. Constructional material comprising a vehicle saturated with fifteen per cent bituminous substance, seventy-five per cent castor oil and ten per cent rape-seed oil, united by gradual heating, and coated with a waterproofing mastic, normally sticky to the touch and lastingly adhesive.
- Signed at Chicago, Illinois, this 9th day of August, 1927.
- ALBERT C. FISCHER.
- 70
- 75
- 80
- 85
- 90
- 95
- 100
- 105
- 110
- 115
- 120
- 125
- 130